



US011268163B2

(12) **United States Patent**  
**Wang et al.**

(10) **Patent No.:** **US 11,268,163 B2**  
(45) **Date of Patent:** **Mar. 8, 2022**

(54) **980 MPa-GRADE HOT-ROLLED  
DUAL-PHASE STEEL AND  
MANUFACTURING METHOD THEREFOR**

(71) **Applicant:** **BAOSHAN IRON & STEEL CO., LTD.**, Shanghai (CN)

(72) **Inventors:** **Huanrong Wang**, Shanghai (CN); **Ana Yang**, Shanghai (CN); **Jiansu Zhang**, Shanghai (CN); **Wei Wang**, Shanghai (CN)

(73) **Assignee:** **BAOSHAN IRON & STEEL CO., LTD.**, Shanghai (CN)

(\*) **Notice:** Subject to any disclaimer, the term of this patent is extended or adjusted under 35 U.S.C. 154(b) by 330 days.

(21) **Appl. No.:** **16/311,376**

(22) **PCT Filed:** **Jun. 19, 2017**

(86) **PCT No.:** **PCT/CN2017/088965**

§ 371 (c)(1),  
(2) Date: **Dec. 19, 2018**

(87) **PCT Pub. No.:** **WO2017/219940**

PCT Pub. Date: **Dec. 28, 2017**

(65) **Prior Publication Data**

US 2019/0233913 A1 Aug. 1, 2019

(30) **Foreign Application Priority Data**

Jun. 21, 2016 (CN) ..... 201610451301.5

(51) **Int. Cl.**  
**C21D 9/46** (2006.01)  
**C22C 38/06** (2006.01)

(Continued)

(52) **U.S. Cl.**  
CPC ..... **C21D 9/46** (2013.01); **C21D 6/005** (2013.01); **C21D 6/008** (2013.01); **C21D 8/0205** (2013.01);

(Continued)

(58) **Field of Classification Search**  
CPC ..... C21D 9/46; C21D 6/005; C21D 6/008;  
C21D 8/0205; C21D 8/0226;  
(Continued)

(56) **References Cited**

U.S. PATENT DOCUMENTS

2009/0214892 A1 8/2009 Kawamura et al.  
2011/0030854 A1\* 2/2011 Matsuda ..... C21D 1/25  
148/504  
2011/0240176 A1\* 10/2011 Kaneko ..... C22C 38/04  
148/503

FOREIGN PATENT DOCUMENTS

GN 101460647 6/2009  
GN 102149841 8/2011  
(Continued)

OTHER PUBLICATIONS

Office Action dated Feb. 4, 2020 for Japanese Patent Application No. 2018-566841.

(Continued)

*Primary Examiner* — John A Hevey

(74) *Attorney, Agent, or Firm* — Lei Fang; Smith Tempel Blaha LLC

(57) **ABSTRACT**

A 980 MPa-grade hot-rolled dual-phase steel and a manufacturing method therefor. The chemical components of the steel comprise, in percentage by weight, 0.10%-0.20% of C, 0.8%-2.0% of Si, 1.0%-2.0% of Mn, 0-0.02% of P, 0-0.005% of S, 0-0.003% of O, 0.02%-0.06% of Al, 0-0.006% of N, 0.01%-0.06% of Nb, 0.01%-0.05% of Ti, and the balance of Fe and inevitable impurities. In addition,

(Continued)



the components need to meet the following relation:  $0.05\% \leq \text{Nb} + \text{Ti} \leq 0.10$ . The microstructure of the steel is made of ferrite and martensite. The average grain size of the ferrite is 5-10  $\mu\text{m}$ , and the equivalent grain size of the martensite is 15-20  $\mu\text{m}$ . The yield strength of the steel is greater than or equal to 500 MPa, the tensile strength of the steel is greater than or equal to 980 MPa, and the ductility  $A_{80}$  is greater than or equal to 12%; the steel has excellent strength, ductility and tenacity matching and a relatively low yield ratio, and can be applied to parts requiring good formability, high strength and reduced thickness, such as wheels.

#### 14 Claims, 2 Drawing Sheets

(51) **Int. Cl.**

*C21D 6/00* (2006.01)  
*C21D 8/02* (2006.01)  
*C22C 38/00* (2006.01)  
*C22C 38/02* (2006.01)  
*C22C 38/04* (2006.01)  
*C22C 38/12* (2006.01)  
*C22C 38/14* (2006.01)

(52) **U.S. Cl.**

CPC ..... *C21D 8/0226* (2013.01); *C21D 8/0263* (2013.01); *C22C 38/001* (2013.01); *C22C 38/002* (2013.01); *C22C 38/02* (2013.01); *C22C 38/04* (2013.01); *C22C 38/06* (2013.01);

*C22C 38/12* (2013.01); *C22C 38/14* (2013.01);  
*C21D 2211/005* (2013.01); *C21D 2211/008* (2013.01)

(58) **Field of Classification Search**

CPC ..... C21D 8/0263; C21D 2211/005; C21D 2211/008; C21D 8/0247; C22C 38/001; C22C 38/002; C22C 38/02; C22C 38/04; C22C 38/12; C22C 38/14; C22C 38/06; B21B 3/00; B21B 37/74

See application file for complete search history.

(56)

#### References Cited

##### FOREIGN PATENT DOCUMENTS

|    |            |         |
|----|------------|---------|
| GN | 106119703  | 11/2016 |
| JP | H05179345  | 7/1993  |
| JP | 2000256778 | 9/2000  |
| JP | 2001192736 | 7/2001  |
| JP | 2007211280 | 8/2007  |
| JP | 2008297609 | 12/2008 |
| JP | 2009084648 | 4/2009  |
| JP | 5379494    | 12/2013 |
| JP | 2014037596 | 2/2014  |

##### OTHER PUBLICATIONS

PCT Patent Application PCT/CN2017/088965 filed on Jun. 19, 2017, International Search Report and Written Opinion dated Dec. 28, 2017.

\* cited by examiner



Fig. 1



Fig. 2



Fig. 3



Fig. 4



Fig. 5

## 1

**980 MPa-Grade Hot-rolled  
Dual-Phase Steel and  
Manufacturing Method Therefor**

**CROSS-REFERENCE TO RELATED  
APPLICATIONS**

This application is a 371 U.S. National Phase of PCT International Application No. PCT/CN2017/088965 filed on Jun. 19, 2017, which claims benefit and priority to Chinese patent application no. 201610451301.5, filed on Jun. 21, 2016. Both of the above-referenced applications are incorporated by reference herein in their entireties.

**TECHNICAL FIELD**

The disclosure pertains to the field of hot-rolled high-strength steel, and particularly relates to a 980 MPa-grade hot-rolled dual-phase steel and a method for manufacturing the same.

**BACKGROUND ART**

Nowadays, carriage wheels of commercial vehicles, especially heavy trucks, are generally manufactured with dual-phase steel. In order to reduce cost, steel wheels are also used for some economical cars (including rims and spokes). Use of high-strength dual-phase steel for manufacturing carriage wheels can reduce wheel weight effectively. For instance, in comparison with common Q345 steel, use of DP600 (i.e. dual-phase steel having a tensile strength of grade 600 MPa) can reduce wheel weight by about 10-15%; and use of DP780 dual-phase steel having a tensile strength of grade 780 MPa can reduce wheel weight by about 5-10% additionally. Dual-phase steel used currently by an overwhelming majority of the domestic carriage wheel manufacturers is mainly low-strength dual-phase steel of 600 MPa or lower. Higher strength dual-phase steel such as DP780 is seldom utilized.

The main reason for wide use of dual-phase steel for carriage wheels of vehicles is that dual-phase steel is inherently characterized by low yield strength, high tensile strength (i.e. low yield ratio), continuous yielding and good processability and formability, etc., as well as relatively good hole expandability. With an eye on the trend of the industrial development, the development of wheel steel is still advancing toward higher strength in general. Moreover, it's common that the strength of the wheel steel utilized today is not high, generally in the range of 500-600 MPa. As national laws and regulations for environmental protection are increasingly stringent, and national measures for limiting vehicle emission are implemented, vehicle weight reduction in the sector of commercial vehicles besides passenger vehicles has already become a trend of the industrial development. In light of such a trend, it's necessary to develop hot-rolled dual-phase steel of higher grades, such as 780 MPa and 980 MPa, to meet the demands of future development of wheel steel. Additionally, high-strength dual-phase steel may also be applied to certain automobile structural members, e.g. automobile frames, anticollision beams, etc.

Currently, high-strength dual-phase steel is mainly grouped into two types: first, cold-rolled high-strength dual-phase steel; second, hot-rolled high-strength dual-phase steel. Cold-rolled high-strength dual-phase steel already has a strength up to 1180 MPa, while the strength of hot-rolled high-strength dual-phase steel has not exceeded 780 MPa.

## 2

This difference between cold-rolled high-strength dual-phase steel and hot-rolled high-strength dual-phase steel arises from some reasons. Firstly, customers' demand for high-strength dual-phase steel focuses mainly on cold-rolled products, while the demand for hot-rolled high-strength dual-phase steel products is weak. Secondly, a hot rolling production line is quite different from a cold rolling production line. A good number of products producible on a cold rolling production line cannot be obtained on a hot rolling production line, unless the composition and process for the steel species are redesigned and optimized. As described above, along with the constant development of the industry, the demand for hot-rolled high-strength dual-phase steel must be increased day by day.

15

**SUMMARY**

One object of the disclosure is to provide a 980 MPa-grade hot-rolled dual-phase steel and a method for manufacturing the same, wherein the hot-rolled dual-phase steel has a yield strength  $\geq 500$  MPa, a tensile strength  $\geq 980$  MPa, and an elongation  $A_{80} \geq 12\%$ . This hot-rolled dual-phase steel shows excellent match between strength, plasticity and toughness, useful for parts requiring good formability, high strength and thinness such as carriage wheels, etc.

To achieve the above object, the technical solution of the disclosure is as follows:

According to the disclosure, a relatively high content of Si is added to guarantee formation of a certain amount of ferrite structure in a limited period of air cooling time after hot rolling, and enlarge the process window for ferrite formation; and Nb and Ti are added in combination mainly for refining austenite grains to the largest extent in a finish rolling stage, such that ferrite formed after phase change is finer, helpful for enhancing a steel plate's strength and plasticity. By precise control over the ferrite and martensite amounts in the structure according to the disclosure, a high-strength ferrite-martensite dual-phase steel having a yield strength  $\geq 500$  MPa and a tensile strength  $\geq 980$  MPa is obtained.

A 980 MPa-grade hot-rolled dual-phase steel, comprising chemical elements in percentage by weight of: C: 0.10-0.20%, Si: 0.8-2.0%, Mn: 1.0-2.0%, P: 0.02%, S: 0.005%, O: 0.003%, Al: 0.02-0.06%, N: 0.006%, Nb: 0.01-0.06%, Ti: 0.01-0.05%, with a balance of Fe and unavoidable impurities, wherein the above elements meet the following relationship:  $0.05\% \leq Nb + Ti \leq 0.10\%$ .

Preferably, in the chemical elements of the hot-rolled dual-phase steel, C: 0.14-0.18% in weight percentage.

Preferably, in the chemical elements of the hot-rolled dual-phase steel, Si: 1.2-1.8% in weight percentage.

Preferably, in the chemical elements of the hot-rolled dual-phase steel, Mn: 1.4-1.8% in weight percentage.

Preferably, in the chemical elements of the hot-rolled dual-phase steel, Nb: 0.03-0.05% in weight percentage.

Preferably, in the chemical elements of the hot-rolled dual-phase steel, Ti: 0.02-0.04% in weight percentage.

Further, the hot-rolled dual-phase steel has a microstructure of ferrite+martensite, wherein the ferrite has a volume fraction of 20-35% and an average grain size of 5-10  $\mu\text{m}$ ; and the martensite has a volume fraction of 65-80% and an equivalent grain size of 15-20  $\mu\text{m}$ .

The hot-rolled dual-phase steel according to the disclosure has a yield strength  $\geq 500$  MPa, a tensile strength  $\geq 980$  MPa and an elongation  $A_{80} \geq 12\%$ .

In the compositional design of the steel according to the disclosure:

Carbon: Carbon is an essential element in the steel, and it's also one of the most important elements in the technical solution of the disclosure. Carbon enlarges an austenite phase zone and stabilizes austenite. As an interstitial atom in the steel, carbon plays an important role for increasing steel strength, and has the greatest influence on the yield strength and tensile strength of the steel. In the disclosure, for the purpose of obtaining a high-strength dual-phase steel having a tensile strength of grade 980 MPa, a carbon content of 0.10% or higher must be ensured. However, the carbon content shall not exceed 0.2%; otherwise, it will be difficult to form a desired amount of ferrite in a two-stage cooling procedure after hot rolling. Therefore, the carbon content in the steel according to the disclosure should be controlled at 0.1-0.2%, preferably 0.14-0.18%.

Silicon: Silicon is an essential element in the steel, and it's also one of the most important elements in the technical solution of the disclosure. The reason for this is that, in order to obtain a high-strength dual-phase steel having a tensile strength of 980 MPa or higher, the size and amount of ferrite shall be controlled on the one hand, and the martensite strength shall be increased on the other hand. This requires suitable increase of carbon and manganese contents in the compositional design. However, both carbon and manganese are elements capable of enlarging an austenite zone and stabilizing austenite. In the very short period of time during air cooling after hot rolling (typically  $\leq 10$  s), it's difficult to form an adequate amount of ferrite. This requires addition of a relatively high content of silicon element. The addition of silicon can obviously promote formation of ferrite, enlarge the process window for ferrite formation, and purify ferrite. At the same time, it can also play a role in part for strengthening. Only when the content of silicon reaches 0.8% or higher can silicon show this effect. Nevertheless, the Si content shall also not be too high; otherwise, the impact toughness of a rolled steel plate will be degraded. Therefore, the silicon content in the steel according to the disclosure is controlled at 0.8-2.0%, preferably 1.2-1.8%.

Manganese: Manganese is also one of the most essential elements in the steel, and it's also one of the most important elements in the technical solution of the disclosure. It's well known that manganese is an important element for enlarging an austenite phase zone, and it can reduce the critical quenching rate of the steel, stabilize austenite, refine grains, and delay transformation of austenite to pearlite. In the present disclosure, in order to guarantee the strength of a steel plate, the manganese content should be controlled at 1.0% or higher. If the manganese content is too low, over-cooled austenite will not be stable enough, and tend to transform into a pearlite type structure during air cooling. Meanwhile, the manganese content shall not exceed 2.0%. If it exceeds 2.0%, not only Mn segregation tends to occur in steel making, but it will also be difficult to form a sufficient amount of ferrite in an air cooling stage after rolling. Moreover, hot cracking tends to occur during continuous casting of slabs. Therefore, the Mn content in the steel according to the disclosure is controlled at 1.0-2.0%, preferably 1.4-1.8%.

Phosphorus: Phosphorus is an impurity element in the steel. Phosphorus has a strong propensity to segregate to a grain boundary. When the phosphorus content in the steel is relatively high ( $\geq 0.1\%$ ),  $\text{Fe}_2\text{P}$  will form and precipitate around the grains, leading to decreased plasticity and toughness of the steel. Therefore, its content should be as low as possible. Generally, it's desirable to control its content within 0.02%, so that the steel making cost will not be increased.

Sulfur: Sulfur is an impurity element in the steel. Sulfur in the steel often combines with manganese to form MnS inclusions. Particularly, when the contents of both sulfur and manganese are relatively high, a large amount of MnS will form in the steel. MnS has certain plasticity itself, and MnS will deform in the rolling direction in a subsequent rolling process, so that the lateral tensile behavior of a steel plate will be degraded. Therefore, the sulfur content in the steel should be as low as possible. In practical production, it's generally controlled within 0.005%.

Aluminum: Aluminum is an additional important alloy element besides the five major elements C, Si, Mn, P, S in the steel. The basic function of aluminum in the disclosure is to remove oxygen in steel making. The aluminum content in the steel is generally not lower than 0.02%. On the other hand, if the aluminum content exceeds 0.06%, its function of refining grains will be degraded. In light of the level at which an aluminum content is controlled in practical production, it's adequate to control the aluminum content in the range of 0.02-0.06% in the steel according to the disclosure.

Nitrogen: Nitrogen is an impurity element in the disclosure, and its content should be as low as possible. Nitrogen is also an unavoidable element in the steel. In typical cases, the amount of residual nitrogen in the steel is generally  $\leq 0.006\%$  if no special controlling measures are taken in steel making. This nitrogen element in a solid dissolved or free form must be immobilized by formation of a nitride. Otherwise, free nitrogen atoms will be very detrimental to the impact toughness of the steel. Furthermore, full-length zig-zag crack defects will easily form in the course of rolling strip steel. In the disclosure, nitrogen atoms are immobilized by addition of titanium element which combines with nitrogen to form stable TiN. Therefore, the nitrogen content in the steel according to the disclosure is controlled within 0.006% and the lower, the better.

Niobium: Niobium is also one of the key elements in the disclosure. It's generally necessary to add a relatively high content of silicon to hot continuously rolled dual-phase steel of 980 MPa or higher grade to promote formation of ferrite phase in rolling and air cooling. However, addition of a high content of silicon will generally increase the brittleness of martensite. Although the carbon content itself is  $\leq 0.20\%$  in the disclosure, after precipitation of a certain amount of ferrite, carbon atoms in the ferrite will be released and enter austenite that has not transformed, such that carbon concentrates in the remaining austenite, and the real carbon content in martensite formed finally is rather high. Martensite has a relatively high brittleness. And the addition of a high content of silicon will further increase the brittleness. Therefore, high silicon type hot-rolled dual-phase steel generally has a low low-temperature impact toughness. In order to maximize the impact toughness of the high silicon type high strength dual-phase steel, a minute amount of niobium is added to the alloy composition in the design to effectively increase the impact toughness of the dual-phase steel by refining grains. The addition of niobium has two effects. First, at a high temperature stage, solid dissolved niobium has a solute drag effect during growth of austenite grains. Second, at a finish rolling stage, niobium carbonitride pins austenite grain boundaries, refines austenite grains, and refines ferrite and martensite transformed finally, so as to enhance the impact toughness of the dual-phase steel. Therefore, the niobium content in the steel according to the disclosure is controlled at 0.01-0.06%, preferably in the range of 0.03-0.05%.

Titanium: Titanium is one of the important elements in the technical solution of the disclosure. Titanium has two major

## 5

effects in the disclosure. First, titanium combines with impurity element nitrogen in the steel to form TiN, so it has an effect of nitrogen immobilization. Second, titanium cooperates with niobium to optimize refining of austenite grains. Free nitrogen atoms in the steel are very disadvantageous to impact toughness of the steel. Addition of a minute amount of titanium can immobilize the free nitrogen. However, the titanium content in the disclosure should not be too high. Otherwise, TiN of a large size may form easily, which is also undesirable for the impact toughness of the steel. As verified by experiments, if Nb is added into the steel alone without addition of Ti, corner cracking tends to form in a continuously cast slab during continuous casting production. Addition of a minute amount of titanium can alleviate the corner cracking problem effectively. Meanwhile, with the proviso that the Nb and Ti contents in the disclosure are controlled in the range of  $0.05\% \leq Nb + Ti \leq 0.10\%$ , the grain refining effect can be achieved well, and the cost is relatively low. Therefore, the titanium content in the steel according to the disclosure is controlled at 0.01-0.05%, preferably in the range of 0.02-0.04%.

Oxygen: Oxygen is an unavoidable element in steel making. For the present disclosure, the oxygen content in the steel is generally 30 ppm or lower after deoxygenation with Al, and thus there is no obvious negative influence on the properties of the steel plate. Therefore, it's acceptable to control the oxygen content in the steel within 30 ppm.

A method for manufacturing the 980 MPa-grade hot-rolled dual-phase steel according to the disclosure, comprising the following steps:

## 1) Smelting and casting

The above chemical composition is smelted, refined and cast into a cast blank or cast billet;

## 2) Heating of the cast blank or cast billet

Heating temperature: 1100-1200° C., heating time: 1-2 hours;

## 3) Hot rolling+staged cooling+cooling

A blooming temperature is 1030-1150° C., wherein 3-5 passes of rough rolling is performed at a temperature of 1000° C. or higher, and an accumulated deformation is  $\geq 50\%$ ; a hold temperature for an intermediate blank is 900-950° C., followed by 3-5 passes of finish rolling with an accumulated deformation  $\geq 70\%$ ; a final rolling temperature is 800-900° C., wherein a steel plate obtained after the final rolling is finished is water cooled to 600-700° C. at a cooling rate  $\geq 100$ ° C./s; after cooled in air for 5-10 seconds, the steel plate is quenched to  $\leq 200$ ° C. at a cooling rate of 30-50° C./s for coiling, and after coiling, a resulting coil is cooled to room temperature at a cooling rate  $\leq 20$ ° C./h.

The manufacture process of the disclosure is designed for the following reasons.

In the design of the rolling process, at a rough rolling stage and a finish rolling stage, the rolling procedure shall be completed as quickly as possible. After the final rolling is finished, rapid cooling is performed at a high cooling rate ( $\geq 100$ ° C./s) to an intermediate temperature at which the cooling is paused. The reason for this is that, if the cooling rate is slow after the rolling is finished, austenite formed inside the steel plate will finish recrystallization in a very short period of time, during which the austenite grains will grow large. When the relatively coarse austenite transforms into ferrite during subsequent cooling, ferrite grains formed along original austenite grain boundaries will be coarse, generally in the range of 10-20  $\mu\text{m}$ , undesirable for improving the strength of the steel plate.

The design concept of the steel plate structures according to the disclosure are fine equiaxed ferrite and martensite

## 6

structures. To achieve a 980 MPa-grade tensile strength, the average grain size of ferrite must be controlled at 10  $\mu\text{m}$  or lower. This requires that, after the final rolling is finished, the steel plate must be cooled rapidly to the desired intermediate temperature at which the cooling is paused. Since the disclosure involves low-carbon steel, there is a great force driving phase change toward ferrite which can form easily. Therefore, after the final rolling, the cooling rate of the strip steel should be quick enough ( $\geq 100$ ° C./s) to avoid formation of ferrite during cooling.

In the staged cooling course according to the disclosure, the cooling-pause temperature in the first stage should be controlled in the range of 600-700° C., for the reason that the strip steel moves quickly in a hot continuous rolling production line, and the length of a water cooling stage is limited, so that it's unlikely to perform air cooling for a long time. The cooling-pause temperature in the first stage should be controlled as far as possible in the optimal temperature range in which ferrite precipitates. The main purpose of the water cooling in the second stage is formation of the desired martensite. The phase change of martensite is a shear type transformation which takes place quickly and can be completed instantaneously, almost having nothing to do with time. As long as the cooling rate reaches the critical cooling rate for martensitic transformation, the phase change of martensite can be completed. Therefore, the water cooling rate in the second stage should be controlled in the range of 30-50° C./s. An unduly high cooling rate may result in excessive stress inside the steel plate, and the strip steel will have a poor plate shape.

A high-strength hot-rolled dual-phase steel having good strength and plasticity can be obtained by the ingenious, reasonable compositional design in coordination with the novel hot rolling process according to the disclosure. The structures of the steel plate are fine ferrite and martensite, wherein the ferrite has a volume fraction of 20-35% and an average grain size of 5-10  $\mu\text{m}$ , and the martensite has a volume fraction of 65-80% and an equivalent grain size of 15-20  $\mu\text{m}$ . In the compositional design, as a result of theoretical analysis and experimental study, the low-yield-ratio, high-strength hot-rolled dual-phase steel having both good plasticity and good impact toughness can be obtained only when the total amount of Nb and Ti meets  $0.05\% \leq Nb + Ti \leq 0.10\%$ , in conjunction with the required rolling process.

The beneficial effects of the disclosure include:

(1) A low-yield-ratio, high-strength hot-rolled dual-phase steel can be manufactured according to the disclosure by adopting a relatively economical compositional design concept in conjunction with an existing hot continuous rolling production line.

(2) A hot-rolled high-strength dual-phase steel plate having a yield strength  $\geq 500$  MPa, a tensile strength  $\geq 980$  MPa, an elongation  $A_{80} \geq 12\%$  and a thickness  $\leq 6$  mm is manufactured according to the disclosure. This steel plate exhibits excellently match between strength, plasticity and toughness, as well as excellent formability. Additionally, it has a relatively low yield ratio. It is useful for parts requiring high strength and thinness such as carriage wheels, etc, and has a promising prospect of applications.

## DESCRIPTION OF THE DRAWINGS

FIG. 1 is a typical metallographical photo of the steel of Example 1 according to the disclosure.

FIG. 2 is a typical metallographical photo of the steel of Example 2 according to the disclosure.

FIG. 3 is a typical metallographical photo of the steel of Example 3 according to the disclosure.

FIG. 4 is a typical metallographical photo of the steel of Example 4 according to the disclosure.

FIG. 5 is a typical metallographical photo of the steel of Example 5 according to the disclosure.

## DETAILED DESCRIPTION

The disclosure will be further illustrated with reference to the following Examples and accompanying drawings.

properties of the steel plates. Ferrite in the structures imparts relatively low yield strength to the plates, while the existence of martensite (having a volume fraction of 65-80%) confers relatively high tensile strength to the steel plates, such that the dual-phase steel according to the disclosure is characterized by good formability and high strength, particularly applicable to fields requiring high strength and small thickness, such as carriage wheels, etc.

As shown by Table 3, a 980 MPa-grade ferrite-martensite dual-phase steel can be manufactured according to the disclosure, wherein the dual-phase steel exhibits a yield strength  $\geq 500$  MPa, a tensile strength  $\geq 980$  MPa, an elongation  $A_{80} \geq 12\%$ , a relatively low yield ratio, and excellent match between strength, plasticity and toughness.

TABLE 1

| unit: weight % |      |      |      |       |        |      |        |       |       |        |
|----------------|------|------|------|-------|--------|------|--------|-------|-------|--------|
|                | C    | Si   | Mn   | P     | S      | Al   | N      | Nb    | Ti    | O      |
| Ex. 1          | 0.20 | 1.95 | 1.10 | 0.010 | 0.0029 | 0.06 | 0.0046 | 0.058 | 0.010 | 0.0029 |
| Ex. 2          | 0.16 | 1.50 | 1.80 | 0.009 | 0.0032 | 0.03 | 0.0042 | 0.035 | 0.015 | 0.0028 |
| Ex. 3          | 0.18 | 1.72 | 1.32 | 0.007 | 0.0028 | 0.06 | 0.0036 | 0.022 | 0.048 | 0.0030 |
| Ex. 4          | 0.11 | 1.05 | 1.99 | 0.009 | 0.0027 | 0.05 | 0.0048 | 0.045 | 0.032 | 0.0029 |
| Ex. 5          | 0.13 | 1.23 | 1.55 | 0.008 | 0.0033 | 0.04 | 0.0044 | 0.011 | 0.050 | 0.0026 |

TABLE 2

| Rolling Process (Steel blank thickness: 120 mm) |                             |                                              |                                               |                                               |                                  |                                    |                                  |                      |                            |                             |                            |     |
|-------------------------------------------------|-----------------------------|----------------------------------------------|-----------------------------------------------|-----------------------------------------------|----------------------------------|------------------------------------|----------------------------------|----------------------|----------------------------|-----------------------------|----------------------------|-----|
| Heating Temperature (° C.)                      | Blooming Temperature (° C.) | Accumulated Deformation By Rough Rolling (%) | Hold Temperature of Intermediate Blank (° C.) | Accumulated Deformation By Finish Rolling (%) | Final Rolling Temperature (° C.) | Post-rolling Cooling Rate (° C./s) | Cooling-pause Temperature (° C.) | Air Cooling Time (s) | Steel Plate Thickness (mm) | Water Cooling Rate (° C./s) | Coiling Temperature (° C.) |     |
| Ex. 1                                           | 1130                        | 1050                                         | 70                                            | 950                                           | 89                               | 900                                | 100                              | 600                  | 10                         | 4                           | 30                         | 200 |
| Ex. 2                                           | 1150                        | 1080                                         | 50                                            | 900                                           | 92                               | 850                                | 120                              | 650                  | 7                          | 5                           | 40                         | 160 |
| Ex. 3                                           | 1200                        | 1150                                         | 65                                            | 930                                           | 90                               | 880                                | 110                              | 670                  | 8                          | 4                           | 35                         | 150 |
| Ex. 4                                           | 1110                        | 1030                                         | 55                                            | 910                                           | 94                               | 800                                | 150                              | 700                  | 5                          | 3                           | 45                         | 180 |
| Ex. 5                                           | 1180                        | 1120                                         | 60                                            | 940                                           | 88                               | 820                                | 130                              | 680                  | 6                          | 6                           | 50                         | 170 |

Table 1 lists the steel compositions in the Examples according to the disclosure; Table 2 lists the manufacture process parameters for the steel in the Examples according to the disclosure; and Table 3 lists the properties of the steel in the Examples according to the disclosure.

The process flow for the Examples according to the disclosure involves: smelting in a converter or electric furnace→secondary refining in a vacuum furnace→casting blank or billet→heating steel blank (billet)→hot rolling+post-rolling staged cooling→coiling steel, wherein the key process parameters are shown in Table 2.

FIGS. 1-5 show the typical metallographical photos of the steel in Examples 1-5 respectively. As can be seen from FIGS. 1-5, the microstructures of the inventive steel plates are fine equiaxed ferrite and martensite (in the figures, the white structure is ferrite, and the dark and grey structures are martensite); ferrite grains are mostly distributed along the original austenite boundaries and have an average grain size of 5-10  $\mu\text{m}$ ; and martensite has an equivalent grain size of about 20  $\mu\text{m}$ . The microstructures correspond well with the

TABLE 3

|       | Yield Strength (MPa) | Tensile Strength (MPa) | Yield Ratio | Elongation ( $A_{80}$ , %) |
|-------|----------------------|------------------------|-------------|----------------------------|
| Ex. 1 | 587                  | 1053                   | 0.56        | 13.0                       |
| Ex. 2 | 561                  | 1046                   | 0.54        | 13.0                       |
| Ex. 3 | 533                  | 1023                   | 0.52        | 13.5                       |
| Ex. 4 | 530                  | 1013                   | 0.52        | 13.0                       |
| Ex. 5 | 562                  | 1064                   | 0.53        | 12.0                       |

What is claimed is:

1. A 980 MPa-grade hot-rolled dual-phase steel, comprising chemical elements in percentage by weight of: C: 0.10-0.20%, Si: 0.8-2.0%, Mn: 1.0-2.0%, P $\leq 0.02\%$ , S $\leq 0.005\%$ , O $\leq 0.003\%$ , Al: 0.02-0.06%, N $\leq 0.006\%$ , Nb: 0.01-0.06%, Ti: 0.01-0.05%, with a balance of Fe and unavoidable impurities, wherein the above elements meet the following relationship:  $0.05\% \leq \text{Nb} + \text{Ti} \leq 0.10\%$ , wherein the hot-rolled dual-phase steel has a microstructure consisting of fine ferrite and as-quenched martensite, wherein the ferrite has a volume fraction of 20-35% and an average grain

size of 5-10  $\mu\text{m}$ ; and the as-quenched martensite has a volume fraction of 65-80% and an equivalent grain size of 15-20  $\mu\text{m}$ .

2. The 980 MPa-grade hot-rolled dual-phase steel according to claim 1, wherein in the chemical elements of the hot-rolled dual-phase steel, C: 0.14-0.18% in weight percentage.

3. The 980 MPa-grade hot-rolled dual-phase steel according to claim 1, wherein in the chemical elements of the hot-rolled dual-phase steel, Si: 1.2-1.8% in weight percentage.

4. The 980 MPa-grade hot-rolled dual-phase steel according to claim 1, wherein in the chemical elements of the hot-rolled dual-phase steel, Mn: 1.4-1.8% in weight percentage.

5. The 980 MPa-grade hot-rolled dual-phase steel according to claim 1, wherein in the chemical elements of the hot-rolled dual-phase steel, Nb: 0.03-0.05% in weight percentage.

6. The 980 MPa-grade hot-rolled dual-phase steel according to claim 1, wherein in the chemical elements of the hot-rolled dual-phase steel, Ti: 0.02-0.04% in weight percentage.

7. The 980 MPa-grade hot-rolled dual-phase steel according to claim 1, wherein the hot-rolled dual-phase steel has a yield strength  $\geq 500$  MPa, a tensile strength  $\geq 980$  MPa and an elongation  $A_{80} \geq 12\%$ .

8. A method for manufacturing the 980 MPa-grade hot-rolled dual-phase steel of claim 1, comprising the following steps:

1) smelting and casting, wherein a chemical composition of claim 1 is smelted, refined and cast into a cast blank or cast billet;

2) heating of the cast blank or cast billet at a heating temperature: 1100-1200° C., heating time: 1-2 hours;

3) hot rolling+staged cooling+coiling, wherein a blooming temperature is 1030-1150° C., wherein 3-5 passes of rough rolling is performed at a temperature of 1000° C. or higher, and an accumulated deformation is  $\geq 50\%$ ;

a hold temperature for an intermediate blank is 900-950° C., followed by 3-5 passes of finish rolling with an accumulated deformation  $\geq 70\%$ ; a final rolling temperature is 800-900° C., wherein a steel plate obtained after the final rolling is finished is water cooled to 600-700° C. at a cooling rate  $\geq 100^\circ \text{C./s.}$ ; after cooled in air for 5-10 seconds, the steel plate is quenched to  $\geq 200^\circ \text{C.}$  at a cooling rate of 30-50° C./s for cooling, and after cooling, a resulting coil is cooled to room temperature at a cooling rate  $\leq 20^\circ \text{C./h.}$

9. The method for manufacturing the 980 MPa-grade hot-rolled dual-phase steel according to claim 8, wherein the hot-rolled dual-phase steel has a microstructure of consisting of fine ferrite and as-quenched martensite, wherein the ferrite has a volume fraction of 20-35% and an average grain size of 5-10  $\mu\text{m}$ ; and the as-quenched martensite has a volume fraction of 65-80% and an equivalent grain size of 15-20  $\mu\text{m}$ .

10. The method for manufacturing the 980 MPa-grade hot-rolled dual-phase steel according to claim 8, wherein the hot-rolled dual-phase steel has a yield strength  $\geq 500$  MPa, a tensile strength  $\geq 980$  MPa and an elongation  $A_{80} \geq 12\%$ .

11. The method for manufacturing the 980 MPa-grade hot-rolled dual-phase steel according to claim 9, wherein the hot-rolled dual-phase steel has a yield strength  $\geq 500$  MPa, a tensile strength  $\geq 980$  MPa and an elongation  $A_{80} \geq 12\%$ .

12. The 980 MPa-grade hot-rolled dual-phase steel according to claim 2, wherein the hot-rolled dual-phase steel has a yield strength  $\geq 500$  MPa, a tensile strength  $\geq 980$  MPa and an elongation  $A_{80} \geq 12\%$ .

13. The 980 MPa-grade hot-rolled dual-phase steel according to claim 3, wherein the hot-rolled dual-phase steel has a yield strength  $\geq 500$  MPa, a tensile strength  $\geq 980$  MPa and an elongation  $A_{80} \geq 12\%$ .

14. The 980 MPa-grade hot-rolled dual-phase steel according to claim 4, wherein the hot-rolled dual-phase steel has a yield strength  $\geq 500$  MPa, a tensile strength  $\geq 980$  MPa and an elongation  $A_{80} \geq 12\%$ .

\* \* \* \* \*